

## 1

3,140,959

### PAPER PRODUCT WITH CHEMICAL WATER-MARK AND MEANS FOR MAKING SAME

Frans V. E. Vaurio, Appleton, Wis., assignor by mesne assignments, to Customark Corporation, Appleton, Wis., a corporation of Wisconsin  
No Drawing. Filed Dec. 27, 1960, Ser. No. 78,228  
8 Claims. (Cl. 117—38)

This invention relates to a paper sheet product with a chemical watermark and means for making same. More in particular this invention relates to means for forming a chemical watermark in otherwise finished paper sheet products which simulates well known watermarked paper sheet products.

Particularly in office operations of commercial enterprises it is often desirable to have writing stationery and other forms of business and professional papers watermarked. Oftentimes business trademarks are watermarked for identity and protective purposes and such watermarking serves as an additional means of distinctiveness associated with a particular business enterprise.

The present practice of watermarking is usually performed during the paper-making process by providing rolls with raised designs interposed usually at a point before the wet paper web enters the dryers. The fibers in the web are displaced in horizontal position and the paper is thus rendered thinner and consequently more transparent in the area of the watermark when viewed under transmitted light. Thus the embossed rolls form the configuration or design of the mark in the damp or wet paper which upon drying remains permanent. After the papermaking and watermarking process is complete the finished paper is cut into sheets of various sizes, such as those established for stationery and the like.

Another known method of forming a watermark involves the employment of a band fitted about a roll and carrying the design or configuration of the water mark in relief. The design of the mark in relief on the band is brought into contact with the wet paper web at the wet presses beyond the Fourdrinier or wet end. At that point the paper is still plastic and compresses readily. The resulting compression of fibres, reducing entrapped air and light refraction, increases the transparency in the area conforming to the configuration of the watermark.

Watermarked paper made as above described has several disadvantages. First the commercial paper making machines are very large and produce paper at a high volume rate. Thus for economical reasons a customer desiring paper bearing a private watermark such as a trademark must purchase a large amount of each kind of paper needed. This of course limits such privately watermarked papers to few but relatively large industrial users or governmental departments as it is obvious that smaller enterprises could not economically purchase and stock a supply sufficient for several years. Second, the cost of the embossed or banded rolls for the paper making machine is obviously extremely high and could therefore not be afforded by smaller industrial users. Third, the cost of setting up the embossed or banded rolls involves both labor as well as loss of production on the paper making machinery which must be taken into account in the net cost to the purchaser. Furthermore, among other disadvantages, the purchaser finds that his private watermark is not positioned uniformly in the finished cut stationery unless he assumes the additional labor cost and paper waste involved in constantly positioning relatively the rolled paper and the cut-off knife. While private watermarks may be formed by presently known methods, it is

## 2

thus clear that orders for paper products so marked must be large if the cost thereof is to be economically justified and orders in small quantities are of such high cost as to be rarely justified.

5 The present invention contemplates the elimination of the above mentioned disadvantages. It is therefore one object of this invention to convert blank paper sheet into a paper sheet product having a uniformly positioned chemical watermark therein conforming to a selected design.

Another object of this invention is to form in a blank cut sheet paper product a visible chemical watermark conforming to a selected design.

A further object of this invention is to form a chemical 15 watermark by impregnating blank paper in the area of the configuration of the mark with a substantially colorless curable thermosetting resin which may or may not be followed by curing the resin.

A still further object of the present invention is to form 20 a chemical watermark according to the preceding objects, wherein the cured resin forming the mark is insoluble in water and ordinary organic solvents.

A yet further object of this invention is to provide 25 blank paper intended for use as paper sheet products with a chemical watermark, according to the preceding objects, wherein the mark may conveniently be positioned uniformly on all sheets.

Another object of this invention is to provide such 30 paper with a chemical watermark, according to the preceding objects, in small quantities at low cost.

Another object of this invention is to provide a method 35 of forming a chemical watermark in paper involving the adequate displacement of entrained air within and between the fibers of the paper.

Another object of the invention is to provide a method 40 of forming a chemical watermark by replacing air entrained in a paper sheet product with a material having an index of refraction reasonably close to that of cellulose.

45 Another object of the invention is to provide a method of forming a chemical watermarked paper sheet product by impregnation thereof within the area of configuration of said mark to replace entrapped air in the area with a substantially colorless thermosetting material curable to insoluble resin at room temperature.

These and other desirable objects inherent in and encompassed by the invention will be more readily understood from the ensuing description and the appended claims.

50 In my previous application for patent filed on August 7, 1959, Serial No. 832,148, now Patent No. 3,085,898, of which this application is a continuation-in-part, there is described numerous novel chemical compositions and method for impregnating blank paper sheet products in 55 the area of the configuration of a selected mark to obtain a simulated watermark. However none of the chemical compositions there described underwent chemical change by reaction. The simulated watermarks thus obtained possessed all the required properties found in watermarks and are essentially permanent in character except that the marks are not resistant to solvent action. Sometimes inks contain solvents which would attack the mark and thus affect adversely its distinctiveness.

60 In the present invention the compositions employed 65 may chemically react to form substantially colorless cured resins which are essentially insoluble in ordinary or common solvents and thus the mark is resistant to solvent action. Thus the major difference between the present application and my above mentioned prior application is the employment of impregnating compositions

which are chemically reactive to form insoluble resins instead of chemically unreactive compositions for use in providing blank paper with a chemical watermark.

The term "chemical watermark" in paper products as herein employed is intended to mean a mark of selected design wherein the area within the configuration of the mark is impregnated with a chemical composition according to this invention resulting in a mark on the paper which substantially meets all of the requirements possessed by a watermark made by the well-known watermarking process. Thus to the consumer the chemical watermark of this invention is indistinguishable from the well known watermark. However since this discussion is directed to those skilled in the art as distinct for the general public the term chemical watermark is used to distinguish the marks obtained according to this invention from the marks obtained by means of the known watermarking methods.

According to this invention blank paper (i.e., having no watermark) is provided with a chemical watermark by impregnating the area of configuration with a novel liquid composition of this invention whereby after curing the liquid resin of the composition to solid, transparent or translucent areas are created in the paper sheet conforming to the desired configuration of the mark. The resulting chemical watermark possesses for all practical purposes the same general physical characteristics in use as a watermark formed by the known processes previously described.

A chemical composition suitable for forming a chemical watermark as above mentioned must have the ability to mark the paper in a manner to render it more translucent or substantially transparent in the impregnated area. Further the chemical composition employed to form the chemical watermark should not alter the surface of the paper adversely. For example it must not render the surface glossy in the impregnated area and must not alter the erasability characteristic of the paper. In addition the chemical composition must withstand aging without substantial discoloration and must not become indistinct through slow migration of the chemicals or otherwise. And of course, the area within the chemical watermark must accept typing, pencilling, printing and writing inks without adverse effects such as feathering or skipping. Certain chemical compositions of this invention have been successfully employed in the formation of chemical watermarks which conform to the above mentioned requirements as hereinafter described.

A conventional watermark, from a fundamental viewpoint, possesses a translucency of higher degree in the area of the mark than that possessed by the paper in the unmarked areas. The most common type of conventional watermark appears more transparent than the surrounding unmarked paper when viewed under transmitted light.

After considerable experimental work it was discovered that soluble resin compositions which were capable of being cured at substantially room temperatures (i.e., 70-90° F.) into insoluble colorless resinous products can be successfully employed to form excellent pseudo-watermarks which possess all of the desired characteristics of watermarks made according to conventional processes. Because a chemical watermark must necessarily be essentially colorless the resin composition must be substantially colorless which requirement precludes the use of many known resins.

Broadly speaking a substantially colorless solution of a curable liquid resin in an organic solvent wherein the resin is curable to a substantially insoluble colorless state may be employed to form chemical watermarks accord-

ing to this invention. Such resins might be cured more

5 rapidly by hardening agents (curing promoters) which may be added to the resin solution provided that the cured resins obtained with the aid of hardening agents remains substantially colorless. Commercial sources of some liquid resins including trade names and manufacturers which were found satisfactory for this invention are shown in Table I below.

TABLE I

|    | Trade Name       | Type                         | Manufacturer                      |
|----|------------------|------------------------------|-----------------------------------|
| 10 | Epon 812         | Epoxy                        | Shell Chemical Co.                |
|    | Dow D.E.R. 332   | do                           | Dow Chemical Co.                  |
|    | Dow D.E.R. 661   | do                           | Do.                               |
| 15 | Dow D.E.R. 664   | do                           | Do.                               |
|    | Dow D.E.R. 667   | do                           | Do.                               |
|    | Maraglas 655     | do                           | Marbette Corp.                    |
|    | Parez 607        | Melamine-formaldehyde.       | American Cyanamid Co.             |
|    | Parez 613        | do                           | Do.                               |
|    | Epoxide 201      | Epoxy                        | Union Carbide Chemicals Co.       |
| 20 | Paraplex P 33    | Polyester                    | Rohm and Haas Co.                 |
|    | ERL 2795         | Epoxy                        | Bakelite Corp.                    |
|    | Araldite 502     | do                           | CIBA Co., Inc.                    |
|    | Epiphene ER-823  | Phenol-formaldehyde-epoxy    | Borden Chemical Co.               |
|    | Uformite F-240   | Butylated urea-formaldehyde. | Rohm and Haas Co.                 |
| 25 | Diepoxide AG-13E | Epoxy                        | Do.                               |
|    | Epoxol 7-4       | do                           | Swift and Co.                     |
|    | Paraplex P-444A  | Polyester                    | Rohm and Haas Co.                 |
|    | Crestoset M      | Urea-formaldehyde            | Crest Chemical Corp.              |
|    | Crestoset M.F.L. | do                           | Do.                               |
|    | Oxiron 2002      | Epoxy                        | Food Machinery and Chemical Corp. |

30 All of the resins in Table I are of the thermosetting type. However, it is understood that the two Paraplex resins are of the polyester type; the Epiphene resin is understood to be of the phenol formaldehyde modified epoxy type; the two Crestoset resins are understood to be of the modified urea formaldehyde type and the remaining resins are understood to be of the epoxy class.

35 Known methods for preparation of epoxy type resins are numerous as shown, for example, in U.S. Patents Nos. 2,444,333; 2,503,726; 2,575,558; 2,582,985; 2,585,115; 2,592,560; 2,694,694; 2,712,535 and 2,864,775. One method for manufacturing an epoxy type resin suitable for use in this invention is the soluble resinous product of the reaction between Bisphenol A (4,4' isopropylidene di-

45 phenol) and epichlorohydrin as indicated below.

The epichlorohydrin and Bisphenol A, usually in a molar proportion of about 10:1, respectively, are placed in a distilling flask, provided with a stirrer and temperature control means, and the flask placed in an inert gas atmosphere such as nitrogen. A reaction period of about 120-150 hours at about 30-50° C. is maintained after which period the temperature is raised to about 80-100° C. and the pressure reduced for the purpose of removing excess epichlorohydrin. The residual intermediate product thus formed is then dissolved in an organic solvent, such as toluene, and an aqueous solution of an inorganic hydroxide (e.g., NaOH) is added slowly with agitation. The amount of inorganic hydroxide added should be slightly in excess of the stoichiometric equivalent to the chlorine present. The resulting mixture is stirred until the reaction is substantially complete. The resinous mass thus obtained is washed with distilled water to remove the inorganic chloride salt formed and excess inorganic hydroxide. The water is then removed by distillation and the residue is a colorless, clear epoxy type liquid resin which is diglycidyl ether of Bisphenol A. The resin thus obtained is a mixture of component compounds having an average molecular weight of about 340-350 and conforming to the following formula:



60 ing to this invention. Such resins might be cured more

65 where  $n$  is zero to about 20 or more.

However it will be apparent from the average molecular weight of about 340-350 that the major proportion of the resin obtained conforms to the above formula when  $n$  equals zero. The epoxy resin obtained has an epoxide equivalent weight of about 173-179 and is curable as explained later herein.

The term "epoxide equivalent weight" means the weight in grams of resin containing one gram equivalent of epoxide. It is usually (but not necessarily) about one-half the average molecular weight as most of these resins are diepoxides.

In the case of Dow D.E.R. 667 epoxy resin the value of  $n$  in the above formula apparently is appreciably above zero as the average molecular weight of this resin is in the range of 3200-4000.

The chemical structure or preparation of most of these proprietary resins apparently are in the nature of trade secrets and thus not available. However it is believed that one or more of the epoxy type resins in Table I are essentially diglycidyl ether of para, para'-isopropylidene-diphenol also known as diglycidyl ether of Bisphenol A formed by reacting epichlorohydrin and Bisphenol A and having the following structural formula.



The Epoxide 201 resin is believed to be a diepoxide, derived from peracetic acid, known as 3,4-epoxy-6-methyl-cyclohexylmethyl - 3,4 - epoxy - 6 - methylcyclohexane - carboxylate of the following structural formula.



Maraglas 655 is believed to be an epoxy resin made by condensing epichlorohydrin and Bisphenol A.

The Epiphen ER 823 resin is believed to be a phenol-formaldehyde novolac resin and epichlorohydrin condensation product of the following structure:



Diepoxyde AG-13E is understood to be bis-epoxydi-cyclopentyl ether of ethylene glycol. Epoxol 7-4 is believed to be epoxidized soybean oil further described in U.S. Patent No. 2,919,283.

Oxiron 2002 is understood to be an epoxidized polyolefin prepared in accordance with U.S. Patents Nos. 2,826,556; 2,833,747; 2,829,131 and 2,829,135.

Aside from the fact that the resin employed must be substantially colorless for making pseudo-watermarks according to this invention it must also possess an index of refraction within critical limits of 1.4 to 1.7 inclusive and the preferred range of limits is 1.45 to 1.65 as measured at 25° C. by conventional method employing the well known Abbe refractometer. This is predicated on the fact that the index of refraction of most cellulose is 1.53-1.55, as obtained by comparison with various organic fluids measured by an Abbe refractometer, and it is desirable to employ a resin having an index of refraction reasonably close to that of the cellulose of the paper to which the chemical watermark is applied according to

this invention. Thus the closer the index of refraction of the resin employed is to the index of refraction of the cellulose, paper the greater amount of parallel light can pass through the paper in the impregnated areas of the chemical watermark which property (i.e., transparency) is most desirable. Conversely the greater the difference between the indexes of refraction results in a corresponding greater amount of diffusion of light. From this it is apparent that if the difference in the indexes of refraction is large the resulting chemical watermark is faint and may be perceived by the eye with difficulty which of course may not be satisfactory. In all of the examples shown later herein as well as Table I the resins employed possessed an index of refraction between 1.4 and 1.7.

Although several types of thermosetting resins of Table I and the resins of the compositions in the examples herein were capable of producing good pseudo-watermarks according to this invention it was observed that the resins of the epoxy class were somewhat superior for this purpose than the other types. The epoxy resins are known to have the ability to protect other polymers from the adverse affects due to aging which is probably due to their ability to react with acid materials. Further, epoxy type resins generally do not possess any particularly obnoxious odors as compared with some other resins.

Accelerated curing of resins of the type indicated in Table I can be effected conveniently by compounds known in the trade as "hardeners" such that the resins will cure at room temperatures (70-90° F.) in reduced time. For purposes of the present invention the cure time for these resins may be as long as two weeks and still be quite satisfactory. Thus short cure time is not necessarily required in this invention. Generally speaking the hardeners may be classed as "curing agents" but not necessarily catalysts. Strictly speaking a true catalyst is not chemically combined with the cured resin as distinct from a compound which accelerates curing but also becomes chemically combined with the cured resin. Both types however, are referred to as "curing agents" because they accelerate the curing rate. In the present invention numerous curing agents or hardeners were employed with successful results. Some of these curing agents found

55 to be satisfactory are shown in Table II by their commercially available trade names and manufacturers.

TABLE II

|                                | Trade Name | Manufacturer                     |
|--------------------------------|------------|----------------------------------|
| Versamid 115                   |            | General Mills Corporation.       |
| Dow D.E.R. Exp. Resin X-2654.4 |            | Dow Chemical Company.            |
| Dow D.E.R. Exp. Resin X-2678.2 |            | Do.                              |
| Shell H-2                      |            | Shell Chemical Company.          |
| DMP-30                         |            | Rohm and Haas Co.                |
| 65 Maraset H655                |            | Marblette Corp.                  |
| Maraset H555                   |            | Do.                              |
| Shell H-1                      |            | Shell Chemical Co.               |
| BF 3-400                       |            | Harshaw Chemical Company.        |
| N-Aminoethyl Piperazine        |            | Jefferson Chemical Company, Inc. |
| Versamid 125                   |            | General Mills Corp.              |
| Cadox MDP                      |            | Cadet Chemical Co.               |
| ERL 2807                       |            | Bakelite Corp.                   |
| Hardener 951                   |            | CIBA Company, Inc.               |
| Hardener EC 20                 |            | Borden Chemical Co.              |
| BF3-Phenol Complex             |            | Allied Chemical Corp.            |
| Eporal                         |            | Roussel Corp.                    |
| Hexahydrophthalic Anhydride    |            | Allied Chemical Corp.            |

Similar as the case of the proprietary resins of Table I most of the chemical formulations for the curing agents of Table II are not available. The Dow D.E.R. Exp. Resin X-2654.4 is believed to be a polyamine. BF<sub>3</sub>-400 is understood to be a complex of boron fluoride with monoethylamine. Eporal is understood to be 4,4'-diaminodiphenyl sulfone. Maraset H655 is characterized as a tertiary amine. The DMP-30 is understood to be 2,4,6-tri(dimethyl aminoethyl) phenol. Other curing agents for epoxy resins found to be satisfactory include diethylene triamine, pyromellitic dianhydride, N-amino ethyl piperazine, methyl nadic anhydride, trimellitic anhydride, dibutyl tin maleate, nadic anhydride, diethylene triamine, diphenyl phosphite, N-acylethanolamine and dipropylene triamine.

All of the curing agents shown in Table II were found suitable for epoxy type resins of Table I except that Cadox MDP is for polyester type resins.

There are numerous known curing agents (hardeners) for epoxy type resins which are described in publications such as "Epoxy Resin" by Skeist (1958), published by Reinhold, New York; "High Polymers," vol. X, Schildknecht (1956), published by Interscience, New York; "Epoxy Resins," by Lee and Neville (1957), published by McGraw-Hill, New York; and U.S. Patents Nos. 2,510,885; 2,548,447 and 2,643,239. In general, polyamines such as diethylenetriamine, triethylenetetramine and xylylenediamine are good curing agents for epoxy type resins. It will be seen from the examples shown herein that the amount of hardener may range from as little as 0.2 percent to as high as about 60 percent by weight where a solvent is not employed and as low as 0.2 percent to as high as about 30 percent by weight when a solvent is employed.

Curing agents found satisfactory for the urea formaldehyde and melamine formaldehyde resins of Table I include maleic anhydride, citric acid, n-butyl acid phosphate, chloroacetic acid, dichloroacetic acid, oxalic acid, mono-n-butyl orthophosphate, sulfamic acid and glacial acetic acid.

In some instances a resin of Table I with or without a curing agent could be satisfactorily used directly to make a chemical watermark according to this invention. However for the most part better results could be obtained if a suitable organic solvent was used with the resin. The solvent employed must, in addition to being a solvent for the resin used, be essentially colorless, non-corrosive to paper, possess a vapor pressure at room temperatures high enough to evaporate with a sufficient rapidity to prevent migration of the resin in paper, possess a vapor pressure low enough to carry the resin into the paper (penetration) prior to evaporation, and, lastly, chemically inert under the conditions employed in this invention.

The solvent preferably should be of the polar type as it appeared that wetting of the paper fibers was better than in the case of non-polar solvents although non-polar solvents can be used as will be seen later. The solvent also must be compatible with the resin selected. If the viscosity of the solution is too low the penetration into the paper is too rapid causing the chemical watermark to be blurred or indistinct. On the other hand if the viscosity of the solution is too high the penetration into the paper is poor and a substantial portion of the resin is deposited on the surface of the paper sheet resulting in a chemical watermark which may have a glossy surface. This is not only undesirable in appearance but may be adversely sensitive to inks. In such case writing inks, for example, do not adhere to the resin surface resulting in "skipping" as is known in the trade. Excessive penetration into the paper results in migration of the resin which tends to make a chemical watermark blurred or indistinct. Table III below lists many solvents which were found to be satisfactory for this invention.

TABLE III

|    |                                           |
|----|-------------------------------------------|
|    | Name:                                     |
| 5  | Methylisobutylketone                      |
|    | Ethyl lactate                             |
|    | Ethylene glycol monomethyl ether          |
|    | Ethylene glycol dimethyl ether            |
|    | Ethylene glycol monoethyl ether           |
| 10 | Ethylene glycol diethyl ether             |
|    | Ethylene glycol monobutyl ether           |
|    | Ethylene glycol monohexyl ether           |
|    | Dibutyl phthalate                         |
| 15 | Diethylene glycol monomethyl ether        |
|    | Diethylene glycol monoethyl ether         |
|    | Diethylene glycol monobutyl ether         |
|    | Diethylene glycol diethyl ether           |
| 20 | Dimethyl formamide                        |
|    | Dimethyl sulfoxide                        |
|    | Triacetin                                 |
|    | Ethylene glycol monoethyl ether acetate   |
|    | N-Butyl acetate                           |
|    | Diethylene glycol monoethyl ether acetate |
|    | Cyclohexanone                             |

In order to evaluate the various compositions of this invention, chemical watermarks of excellent quality were obtained in the laboratory by hand impregnation. The hand impregnation was accomplished by depositing a small metered amount (e.g., 1 to 2 grams) of the composition on the surface of a foot-square piece of one-quarter inch thick plate glass. The liquid composition was spread uniformly over the glass surface with a conventional handproofer consisting of an engraved roll bearing 75 depressions per inch and fitted with a handle. A die or hand stamp of rubber-like material having inscribed in relief on the face thereof a design or configuration conforming to a typical watermark was pressed against the wet film of the composition and then stamped on the paper sheet. The chemical watermarked paper sheet was allowed to dry and cure at ambient room temperatures (70°-90° F.) and then examined. Thus chemical watermarks were applied to paper sheets much in the same manner as one would rubber stamp paper using an inked pad except instead of ink the compositions of this invention were used.

Where curing agents were employed the time required for the resin to cure at ambient room temperatures to a degree sufficient to resist solubility in 95% ethanol or acetone varied somewhat depending on the particular resin used. However all resins with curing agents of the compositions employed in the various examples shown later herein cured satisfactorily with reference to ethanol or acetone solubility in periods less than two weeks at ambient room temperatures.

Testing for cure of the resin in the chemical watermark made by laboratory hand stamping as above described was made by agitating the paper sheet bearing the chemical watermark in the solvent (e.g., ethanol) for a period of two minutes at room temperature. If the solvent extracted resin the chemical watermark disappeared. Where, on the other hand, the chemical watermark remained after agitation in the solvent this indicated that the resin cured to a solvent resistant state.

The two week curing time requirement is generally not objectionable because packing and shipping operations for paper stationery together with upacking and use by the customer usually is at least this long. Of course if desired the curing rate of the resin can be greatly accelerated by heating the chemical watermarked paper to 70°-90° C. for a period of about one hour without discoloring the paper.

By way of illustration of the invention, excellent chemical watermarks were obtained by laboratory hand impregnation, as above described, employing novel compositions of this invention in each of the following examples, the stated proportions being in terms of weight.

## Example 1

Dow D.E.R. 332 ----- 60 grams, 33%.  
 Dow Hardener X-2654.4 ----- 12 grams, 7%.  
 Ethyleneglycol monomethyl ether ----- 108 grams, 60%.

## Example 2

Dow D.E.R. 332 ----- 100 grams, 58%.  
 Dow Hardener X-2654.4 ----- 20 grams, 12%.  
 Ethyleneglycol monomethyl ether ----- 51.4 grams, 30%.

## Example 3

Dow D.E.R. 332 ----- 100 grams, 66%.  
 Dow Hardener X-2654.4 ----- 20 grams, 13%.  
 Ethyleneglycol monomethyl ether ----- 32 grams, 21%.

## Example 4

Dow D.E.R. 332 ----- 60 grams, 33%.  
 Dow Hardener X-2654.4 ----- 12 grams, 7%.  
 Diethyleneglycol monoethyl ether ----- 108 grams, 60%.

## Example 5

Dow D.E.R. 332 ----- 100 grams, 58%.  
 Dow Hardener X-2654.4 ----- 20 grams, 12%.  
 Diethyleneglycol monoethyl ether ----- 51.4 grams, 30%.

## Example 6

Dow D.E.R. 332 ----- 60 grams, 33%.  
 Dow Hardener X-2654.4 ----- 12 grams, 7%.  
 Diethyleneglycol diethyl ether ----- 108 grams, 60%.

## Example 7

Dow D.E.R. 332 ----- 100 grams, 58%.  
 Dow Hardener X-2654.4 ----- 20 grams, 12%.  
 Diethyleneglycol diethyl ether ----- 51.4 grams, 30%.

## Example 8

Dow D.E.R. 332 ----- 60 grams, 33%.  
 Dow Hardener X-2654.4 ----- 12 grams, 7%.  
 Diethyleneglycol monobutyl ether ----- 108 grams, 60%.

## Example 9

Dow D.E.R. 332 ----- 100 grams, 58%.  
 Dow Hardener X-2654.4 ----- 20 grams, 12%.  
 Diethyleneglycol monobutyl ether ----- 51.4 grams, 30%.

## Example 10

Dow D.E.R. 332 ----- 60 grams, 33%.  
 Dow Hardener X-2654.4 ----- 12 grams, 7%.  
 Ethyleneglycol monoethyl ether acetate ----- 108 grams, 60%.

## Example 11

Dow D.E.R. 332 ----- 100 grams, 58%.  
 Dow Hardener X-2654.4 ----- 20 grams, 12%.  
 Ethyleneglycol monoethyl ether acetate ----- 51.4 grams, 30%.

## Example 12

Dow D.E.R. 332 ----- 60 grams, 33%.  
 Dow Hardener X-2654.4 ----- 12 grams, 7%.  
 Methyl isobutyl ketone ----- 108 grams, 60%.

## Example 13

Dow D.E.R. 332 ----- 100 grams, 58%.  
 Dow Hardener X-2654.4 ----- 20 grams, 12%.  
 Methyl isobutyl ketone ----- 51.4 grams, 30%.

## Example 14

Dow D.E.R. 332 ----- 60 grams, 33%.  
 Dow Hardener X-2654.4 ----- 12 grams, 7%.  
 Dimethyl formamide ----- 108 grams, 60%.

## Example 15

Dow D.E.R. 332 ----- 100 grams, 58%.  
 Dow Hardener X-2654.4 ----- 20 grams, 12%.  
 Dimethyl formamide ----- 51.4 grams, 30%.

## Example 16

Dow D.E.R. 332 ----- 60 grams, 33%.  
 Dow Hardener X-2654.4 ----- 12 grams, 7%.  
 Dimethyl sulfoxide ----- 108 grams, 60%.

5

10

## Example 17

Dow D.E.R. 332 ----- 100 grams, 58%.  
 Dow Hardener X-2654.4 ----- 20 grams, 12%.  
 Dimethyl sulfoxide ----- 51.4 grams, 30%.

15

## Example 18

Dow D.E.R. 332 ----- 60 grams, 33%.  
 Dow Hardener X-2654.4 ----- 12 grams, 7%.  
 Ethyleneglycol monoethyl ether ----- 108 grams, 60%.

20

## Example 19

Dow D.E.R. 332 ----- 100 grams, 58%.  
 Dow Hardener X-2654.4 ----- 20 grams, 12%.  
 Ethyleneglycol monoethyl ether ----- 51.4 grams, 30%.

25

## Example 20

Dow D.E.R. 332 ----- 60 grams, 33%.  
 Dow Hardener X-2654.4 ----- 12 grams, 7%.  
 Ethyleneglycol monomethyl ether ----- 108 grams, 60%.

30

## Example 21

Dow D.E.R. 332 ----- 100 grams, 58%.  
 Dow Hardener X-2654.4 ----- 20 grams, 12%.  
 Ethyleneglycol monomethyl ether ----- 51.4 grams, 30%.

35

## Example 22

Dow D.E.R. 332 ----- 60 grams, 33%.  
 Dow Hardener X-2654.4 ----- 12 grams, 7%.  
 Ethyleneglycol monobutyl ether ----- 108 grams, 60%.

40

## Example 23

Dow D.E.R. 332 ----- 100 grams, 58%.  
 Dow Hardener X-2654.4 ----- 20 grams, 12%.  
 Ethyleneglycol monobutyl ether ----- 51.4 grams, 30%.

45

## Example 24

Dow D.E.R. 332 ----- 60 grams, 33%.  
 Dow Hardener X-2654.4 ----- 12 grams, 7%.  
 Ethyleneglycol monohexyl ether ----- 108 grams, 60%.

50

## Example 25

Dow D.E.R. 332 ----- 100 grams, 58%.  
 Dow Hardener X-2654.4 ----- 20 grams, 12%.  
 Ethyleneglycol monohexyl ether ----- 51.4 grams, 30%.

55

The foregoing examples illustrates the wide range of solvent content in the compositions which can be satisfactorily employed. In some instances a solvent was omitted with satisfactory results as shown later herein and in other instances a solvent concentration as high as 80% produced satisfactory results. Of course in commercial operations the particular solvent used and content thereof in the composition for best results will depend to some extent on the type of commercial printing press used and conditions of operation as well as the characteristics of the paper to which a chemical watermark is to be imprinted in accordance with this invention.

60

The following immediate group of examples illustrates several compositions all of which produced excellent chemical watermarks according to this invention. Some of these compositions have been employed using commercial printing machinery and in each case excellent chemical watermarks were obtained.

65

## Example 26

Percent

Epon 812 (resin) ----- 57.1  
 Versamid 115 (hardener) ----- 28.6  
 Diethyleneglycol monomethyl ether ----- 14.3

70

75

11  
Example 27

|                                   | Percent |
|-----------------------------------|---------|
| Dow D.E.R. 332 (resin)            | 44.5    |
| Dow Hardener X-2654.4             | 11.0    |
| Diethyleneglycol monomethyl ether | 44.5    |

## Example 28

|                                   |      |
|-----------------------------------|------|
| Dow D.E.R. 332 (resin)            | 40.0 |
| Dow Hardener X-2654.4             | 20.0 |
| Diethyleneglycol monomethyl ether | 40.0 |

## Example 29

|                                   |      |
|-----------------------------------|------|
| Dow D.E.R. 332 (resin)            | 33.4 |
| Dow Hardener X-2654.4             | 33.3 |
| Diethyleneglycol monomethyl ether | 33.3 |

## Example 30

|                                   |      |
|-----------------------------------|------|
| Maraglas 655 (resin)              | 40.0 |
| Dow Hardener X-2654.4             | 20.0 |
| Diethyleneglycol monomethyl ether | 40.0 |

## Example 31

|                      |      |
|----------------------|------|
| Maraglas 655 (resin) | 66.7 |
| Shell H-2 (hardener) | 33.3 |

## Example 32

|                      |      |
|----------------------|------|
| Epon 812 (resin)     | 50.0 |
| Shell H-2 (hardener) | 50.0 |

## Example 33

|                                   |      |
|-----------------------------------|------|
| Epon 812 (resin)                  | 40.0 |
| Dow Hardener X-2654.4             | 20.0 |
| Diethyleneglycol monomethyl ether | 40.0 |

## Example 34

|                                   |      |
|-----------------------------------|------|
| Epon 812 (resin)                  | 33.4 |
| Dow Hardener X-2654.4             | 33.3 |
| Diethyleneglycol monomethyl ether | 33.3 |

|                  |      |
|------------------|------|
| Epon 812 (resin) | 90.9 |
| DMP-30           | 9.1  |

## Example 36

|                                   |      |
|-----------------------------------|------|
| Dow D.E.R. 332 (resin)            | 65.6 |
| Ethylene triamine (hardener)      | 1.6  |
| Diethyleneglycol monomethyl ether | 32.8 |

## Example 37

|                                   |      |
|-----------------------------------|------|
| Dow D.E.R. 332                    | 41.7 |
| Dow Hardener X-2654.4             | 16.6 |
| Diethyleneglycol monomethyl ether | 41.7 |

## Example 38

|                                   |      |
|-----------------------------------|------|
| Dow D.E.R. 332 (resin)            | 43.5 |
| Dow Hardener X-2654.4             | 13.0 |
| Diethyleneglycol monomethyl ether | 43.5 |

## Example 39

|                                   |      |
|-----------------------------------|------|
| Dow D.E.R. 332 (resin)            | 45.5 |
| Dow Hardener X-2654.4             | 9.0  |
| Diethyleneglycol monomethyl ether | 45.5 |

## Example 40

|                                   |      |
|-----------------------------------|------|
| Dow D.E.R. 332 (resin)            | 47.6 |
| Dow Hardener X-2654.4             | 4.8  |
| Diethyleneglycol monomethyl ether | 47.6 |

## Example 41

|                                   |      |
|-----------------------------------|------|
| Dow D.E.R. 332 (resin)            | 40.0 |
| Pyromellitic anhydride (hardener) | 20.0 |
| Diethyleneglycol monomethyl ether | 40.0 |

## Example 42

|                                   |      |
|-----------------------------------|------|
| Parez 607 (resin)                 | 33.3 |
| Diethyleneglycol monomethyl ether | 66.7 |

12  
Example 43

|                                   | Percent |
|-----------------------------------|---------|
| Dow D.E.R. 332 (resin)            | 49.9    |
| Dow Hardener X-2654.4             | 0.2     |
| Diethyleneglycol monomethyl ether | 49.9    |

## Example 44

|                                   |      |
|-----------------------------------|------|
| Dow D.E.R. 332 (resin)            | 48.9 |
| Dow Hardener X-2654.4             | 2.2  |
| Diethyleneglycol monomethyl ether | 48.9 |

## Example 45

|                     |      |
|---------------------|------|
| ERL 2795 (resin)    | 99.5 |
| ERL 2807 (hardener) | 0.5  |

## Example 46

|                     |      |
|---------------------|------|
| ERL 2795 (resin)    | 97.6 |
| ERL 2807 (hardener) | 2.4  |

## Example 47

|                     |      |
|---------------------|------|
| ERL 2795 (resin)    | 95.2 |
| ERL 2807 (hardener) | 4.8  |

## Example 48

|                                   |      |
|-----------------------------------|------|
| Maraglas 655 (resin)              | 57.4 |
| Dow Hardener X-2654.4             | 14.4 |
| Diethyleneglycol monomethyl ether | 28.2 |

## Example 49

|                                   |      |
|-----------------------------------|------|
| Maraglas 655 (resin)              | 44.5 |
| Dow Hardener X-2654.4             | 11.0 |
| Diethyleneglycol monomethyl ether | 44.5 |

## Example 50

|                      |      |
|----------------------|------|
| Maraglas 655 (resin) | 99.0 |
| Shell H-1 (hardener) | 1.0  |

## Example 51

|                                   |      |
|-----------------------------------|------|
| Maraglas 655 (resin)              | 48.8 |
| Shell H-1 (hardener)              | 2.4  |
| Diethyleneglycol monomethyl ether | 48.8 |

## Example 52

|                                   |      |
|-----------------------------------|------|
| Maraglas 655 (resin)              | 62.6 |
| Shell H-1 (hardener)              | 6.2  |
| Diethyleneglycol monomethyl ether | 31.2 |

## Example 53

|                                   |      |
|-----------------------------------|------|
| Maraglas 655 (resin)              | 50.0 |
| Shell H-1 (hardener)              | 25.0 |
| Diethyleneglycol monomethyl ether | 25.0 |

## Example 54

|                                   |      |
|-----------------------------------|------|
| Maraglas 655 (resin)              | 64.6 |
| Shell H-2 (hardener)              | 3.2  |
| Diethyleneglycol monomethyl ether | 32.2 |

## Example 55

|                                   |      |
|-----------------------------------|------|
| Maraglas 655 (resin)              | 62.6 |
| Shell H-2 (hardener)              | 6.2  |
| Diethyleneglycol monomethyl ether | 31.2 |

## Example 56

|                                   |      |
|-----------------------------------|------|
| Maraglas 655 (resin)              | 50.0 |
| Shell H-2                         | 25.0 |
| Diethyleneglycol monomethyl ether | 25.0 |

## Example 57

|                      |      |
|----------------------|------|
| Epon 812 (resin)     | 66.7 |
| Shell H-2 (hardener) | 33.3 |

## Example 58

|                                   |      |
|-----------------------------------|------|
| Epon 812 (resin)                  | 45.4 |
| Dow Hardener X-2654.4             | 9.2  |
| Diethyleneglycol monomethyl ether | 45.4 |

13

Example 59

|                                   | Percent |
|-----------------------------------|---------|
| Epon 812 (resin)                  | 40.0    |
| Dow Hardener X-2654.4             | 20.0    |
| Diethyleneglycol monomethyl ether | 40.0    |

Example 60

|                   |      |
|-------------------|------|
| Epon 812 (resin)  | 95.2 |
| DMP 30 (hardener) | 4.8  |

Example 61

|                   |      |
|-------------------|------|
| Epon 812 (resin)  | 83.3 |
| DMP 30 (hardener) | 16.7 |

Example 62

|                                   |      |
|-----------------------------------|------|
| Araldite 502 (resin)              | 74.1 |
| Hardener 951                      | 7.4  |
| Diethyleneglycol monomethyl ether | 18.5 |

Example 63

|                                   |      |
|-----------------------------------|------|
| Epiphene ER-823 (resin)           | 45.5 |
| Hardener EC-20                    | 9.0  |
| Diethyleneglycol monomethyl ether | 45.5 |

Example 64

|                                   |      |
|-----------------------------------|------|
| Parez 613 (resin)                 | 30.4 |
| Dow D.E.R. 332 (resin)            | 21.9 |
| Dow Hardener X-2654.4             | 10.9 |
| Chloroacetic acid (hardener)      | 2.2  |
| Diethyleneglycol monomethyl ether | 34.6 |

Example 65

|                        |    |
|------------------------|----|
| Dow D.E.R. 332 (resin) | 50 |
| Methyl nadic anhydride | 50 |

Example 66

|                        |      |
|------------------------|------|
| Dow D.E.R. 332 (resin) | 41.6 |
| Methyl nadic anhydride | 58.4 |

Example 67

|                        |      |
|------------------------|------|
| Dow D.E.R. 332 (resin) | 33.3 |
| Methyl nadic anhydride | 66.7 |

Example 68

|                                 |      |
|---------------------------------|------|
| Dow D.E.R. 332 (resin)          | 48.1 |
| BF <sub>3</sub> -400 (hardener) | 3.8  |
| Methyl nadic anhydride          | 48.1 |

Example 69

|                       |      |
|-----------------------|------|
| Maraglas 655 (resin)  | 93.0 |
| Maraset Hardener H555 | 7.0  |

Example 70

|                       |      |
|-----------------------|------|
| Maraglas 655 (resin)  | 90.9 |
| Maraset Hardener H555 | 9.1  |

Example 71

|                       |    |
|-----------------------|----|
| Maraglas 655 (resin)  | 77 |
| Maraset Hardener H555 | 23 |

Example 72

|                       |    |
|-----------------------|----|
| Maraglas 655 (resin)  | 50 |
| Maraset Hardener H555 | 50 |

Example 73

|                                   |      |
|-----------------------------------|------|
| Dow D.E.R. 332 (resin)            | 47.6 |
| Pyromellitic anhydride            | 4.8  |
| Diethyleneglycol monomethyl ether | 47.6 |

Example 74

|                                   |    |
|-----------------------------------|----|
| Dow D.E.R. 332 (resin)            | 40 |
| Pyromellitic anhydride            | 20 |
| Diethyleneglycol monomethyl ether | 40 |

Example 75

|                                   |    |
|-----------------------------------|----|
| Dow D.E.R. 332 (resin)            | 56 |
| BF <sub>3</sub> -400              | 4  |
| Diethyleneglycol monomethyl ether | 40 |

14

Example 76

|                                   | Percent |
|-----------------------------------|---------|
| Dow D.E.R. 332 (resin)            | 69      |
| N-Aminoethyl Piperazine           | 10      |
| Diethyleneglycol monomethyl ether | 21      |

Example 77

|                                   |    |
|-----------------------------------|----|
| Dow D.E.R. 332 (resin)            | 72 |
| N-Aminoethyl Piperazine           | 7  |
| Diethyleneglycol monomethyl ether | 21 |

Example 78

|                                   |      |
|-----------------------------------|------|
| Dow D.E.R. 332 (resin)            | 66.7 |
| N-Aminoethyl Piperazine           | 13.3 |
| Diethyleneglycol monomethyl ether | 20.0 |

Example 79

|                                   |      |
|-----------------------------------|------|
| Dow D.E.R. 332 (resin)            | 64.6 |
| N-Aminoethyl Piperazine           | 16.1 |
| Diethyleneglycol monomethyl ether | 19.3 |

Example 80

|                                   |      |
|-----------------------------------|------|
| Dow D.E.R. 332 (resin)            | 45.5 |
| Eporal (hardener)                 | 9.0  |
| Diethyleneglycol monomethyl ether | 45.5 |

Example 82

|                                            |      |
|--------------------------------------------|------|
| Dow D.E.R. 332 (resin)                     | 58.6 |
| BF <sub>3</sub> -Phenol Complex (hardener) | 0.3  |
| Diethyleneglycol monomethyl ether          | 41.1 |

Example 83

|                                            |      |
|--------------------------------------------|------|
| Dow D.E.R. 332 (resin)                     | 35.5 |
| Hexahydrophthalic Anhydride (hardener)     | 28.8 |
| BF <sub>3</sub> -Phenol Complex (hardener) | 0.2  |
| Diethyleneglycol monomethyl ether          | 35.5 |

Example 84

|                                            |      |
|--------------------------------------------|------|
| Dow D.E.R. 332 (resin)                     | 41.5 |
| Hexahydrophthalic Anhydride (hardener)     | 16.7 |
| BF <sub>3</sub> -Phenol Complex (hardener) | 0.3  |
| Diethyleneglycol monomethyl ether          | 41.5 |

Example 85

|                                            |      |
|--------------------------------------------|------|
| Dow D.E.R. 332 (resin)                     | 45.3 |
| BF <sub>3</sub> -Phenol Complex (hardener) | 0.3  |
| Hexahydrophthalic Anhydride (hardener)     | 9.1  |
| Diethyleneglycol monomethyl ether          | 45.3 |

Example 86

|                                                |      |
|------------------------------------------------|------|
| Dow D.E.R. 332 (resin)                         | 58.6 |
| BF <sub>3</sub> -Piperidine Complex (hardener) | 0.3  |
| Diethyleneglycol monomethyl ether              | 41.1 |

Example 87

|                                                |      |
|------------------------------------------------|------|
| Dow D.E.R. 332 (resin)                         | 58.5 |
| BF <sub>3</sub> -Piperidine Complex (hardener) | 0.6  |
| Diethyleneglycol monomethyl ether              | 40.9 |

Example 88

|                                                |      |
|------------------------------------------------|------|
| Dow D.E.R. 332 (resin)                         | 58.3 |
| BF <sub>3</sub> -Piperidine Complex (hardener) | 0.9  |
| Diethyleneglycol monomethyl ether              | 40.8 |

Example 89

|                                                |      |
|------------------------------------------------|------|
| Dow D.E.R. 332 (resin)                         | 57.8 |
| BF <sub>3</sub> -Piperidine Complex (hardener) | 1.7  |
| Diethyleneglycol monomethyl ether              | 40.5 |

Example 90

|                                                |      |
|------------------------------------------------|------|
| Dow D.E.R. 332 (resin)                         | 55.6 |
| BF <sub>3</sub> -Piperidine Complex (hardener) | 5.6  |
| Diethyleneglycol monomethyl ether              | 38.8 |

## 15

In the preceding five examples the  $\text{BF}_3$ -Piperidine Complex is commercially available but may be prepared by bubbling boron trifluoride in piperidine at room temperature.

## Example 91

|                                          | Percent |
|------------------------------------------|---------|
| Dow D.E.R. 332 (resin)                   | 58.3    |
| $\text{BF}_3$ -Phenol Complex (hardener) | 0.8     |
| Diethyleneglycol monomethyl ether        | 40.9    |

## Example 92

|                                          | Percent |
|------------------------------------------|---------|
| Dow D.E.R. 332 (resin)                   | 58.2    |
| $\text{BF}_3$ -Phenol Complex (hardener) | 1.2     |
| Diethyleneglycol monomethyl ether        | 40.6    |

## Example 93

|                                          | Percent |
|------------------------------------------|---------|
| Dow D.E.R. 332 (resin)                   | 33      |
| Crestoset M (resin)                      | 33      |
| $\text{BF}_3$ -Phenol Complex (hardener) | 1       |
| Diethyleneglycol monomethyl ether        | 33      |

## Example 94

|                                   | Percent |
|-----------------------------------|---------|
| Dow D.E.R. 661 (resin)            | 29.6    |
| Dow D.E.R. X-2673.2 (hardener)    | 7.4     |
| N-Aminoethyl Piperazine           | 3.0     |
| Diethyleneglycol monomethyl ether | 60.0    |

## Example 95

|                                   | Percent |
|-----------------------------------|---------|
| Dow D.E.R. 664 (resin)            | 29.6    |
| Dow D.E.R. X-2673.2 (hardener)    | 7.4     |
| N-Aminoethyl Piperazine           | 3.0     |
| Diethyleneglycol monomethyl ether | 60.0    |

## Example 96

|                                   | Percent |
|-----------------------------------|---------|
| Dow D.E.R. 667 (resin)            | 29.6    |
| Dow D.E.R. X-2673.2 (hardener)    | 7.4     |
| N-Aminoethyl Piperazine           | 3.0     |
| Diethyleneglycol monomethyl ether | 60.0    |

## Example 97

|                                   | Percent |
|-----------------------------------|---------|
| Crestoset M (resin)               | 50      |
| Oxalic acid (hardener)            | 5       |
| Diethyleneglycol monomethyl ether | 45      |

## Example 98

|                                  | Percent |
|----------------------------------|---------|
| Crestoset M (resin)              | 50      |
| Oxalic acid (hardener)           | 5       |
| Diethyleneglycol monobutyl ether | 45      |

## Example 99

|                        | Percent |
|------------------------|---------|
| Crestoset M (resin)    | 50      |
| Oxalic acid (hardener) | 5       |
| Diacetin               | 45      |

## Example 100

|                        | Percent |
|------------------------|---------|
| Crestoset M (resin)    | 50      |
| Oxalic acid (hardener) | 5       |
| Monacetin              | 45      |

## Example 101

|                        | Percent |
|------------------------|---------|
| Crestoset M (resin)    | 50      |
| Oxalic acid (hardener) | 5       |
| Dipropylene glycol     | 45      |

## Example 102

|                                   | Percent |
|-----------------------------------|---------|
| Crestoset M (resin)               | 50      |
| Citric acid (hardener)            | 5       |
| Diethyleneglycol monomethyl ether | 45      |

## Example 103

|                                  | Percent |
|----------------------------------|---------|
| Crestoset M (resin)              | 50      |
| Citric acid (hardener)           | 5       |
| Diethyleneglycol monobutyl ether | 45      |

## Example 104

|                        | Percent |
|------------------------|---------|
| Crestoset M (resin)    | 50      |
| Citric acid (hardener) | 5       |
| Diacetin               | 45      |

## 16

## Example 105

|                     | Percent |
|---------------------|---------|
| Crestoset M (resin) | 50      |
| Citric acid         | 5       |
| Monacetin           | 45      |

## Example 106

|                     | Percent |
|---------------------|---------|
| Crestoset M (resin) | 50      |
| Citric acid         | 5       |
| Dipropylene glycol  | 45      |

## Example 107

|                                   | Percent |
|-----------------------------------|---------|
| Crestoset M (resin)               | 38.4    |
| Phosphoric acid                   | 3.8     |
| Diethyleneglycol monomethyl ether | 57.8    |

## Example 108

|                                   | Percent |
|-----------------------------------|---------|
| Crestoset M (resin)               | 62.5    |
| Citric acid (hardener)            | 6.2     |
| Diethyleneglycol monomethyl ether | 31.3    |

## Example 109

|                        | Percent |
|------------------------|---------|
| Crestoset M (resin)    | 43.4    |
| Citric acid (hardener) | 4.3     |
| Diacetin               | 52.3    |

## Example 111

|                        | Percent |
|------------------------|---------|
| Crestoset M (resin)    | 56.2    |
| Citric acid (hardener) | 5.6     |
| Monacetin              | 38.2    |

## Example 112

|                                 | Percent |
|---------------------------------|---------|
| Crestoset M (resin)             | 50      |
| Oxalic acid                     | 5       |
| Ethylene glycol monohexyl ether | 45      |

In all of the preceding examples a curing agent (hardener) was employed to cure the resin but in some instances a solvent was omitted. As mentioned previously a solvent is not always required. Some of the resins require the presence of a solvent and the amount of solvent employed is governed to an appreciable extent by the impregnating characteristics of the paper to be chemical watermarked in accordance with this invention.

In the following examples a curing agent is omitted. The resin will not cure on contact with the air at ambient temperature. However where curing is desired in the case of chemical watermarking according to this invention the time required to cure the resin to an organic solvent resistant state is not too important for, as previously mentioned, a period of two or more weeks usually elapses between chemical watermarking and the time when the customer receives the product. Thus the following examples illustrate compositions which use results in excellent chemical watermarks according to this invention without employing curing agents.

## Example 113

|                                   | Percent |
|-----------------------------------|---------|
| Dow D.E.R. 332 (resin)            | 65      |
| Diethyleneglycol monomethyl ether | 35      |

## Example 114

|                                   | Percent |
|-----------------------------------|---------|
| Dow D.E.R. 332 (resin)            | 80      |
| Diethyleneglycol monomethyl ether | 20      |

## Example 115

|                        | Percent |
|------------------------|---------|
| Dow D.E.R. 332 (resin) | 30      |
| Cyclohexanone          | 70      |

## Example 116

|                        | Percent |
|------------------------|---------|
| Dow D.E.R. 332 (resin) | 80      |
| Cyclohexanone          | 20      |

17

Example 117

Percent

|                              |    |
|------------------------------|----|
| Dow D.E.R. 332 (resin) ----- | 80 |
| Monoacetin -----             | 20 |

Example 118

5

|                              |    |
|------------------------------|----|
| Dow D.E.R. 332 (resin) ----- | 80 |
| Diacetin -----               | 20 |

Example 119

10

|                              |    |
|------------------------------|----|
| Dow D.E.R. 332 (resin) ----- | 30 |
| Triacetin -----              | 70 |

Example 120

15

|                                        |    |
|----------------------------------------|----|
| Dow D.E.R. 332 (resin) -----           | 80 |
| Diethyleneglycol monohexyl ether ----- | 20 |

Example 121

20

|                              |    |
|------------------------------|----|
| Dow D.E.R. 332 (resin) ----- | 90 |
| Dimethyl sulfoxide -----     | 10 |

Example 122

25

|                              |    |
|------------------------------|----|
| Dow D.E.R. 332 (resin) ----- | 80 |
| Dibutyl phthalate -----      | 20 |

Example 123

30

|                                        |    |
|----------------------------------------|----|
| Dow D.E.R. 332 (resin) -----           | 40 |
| Diethyleneglycol monobutyl ether ----- | 60 |

Example 124

35

|                              |    |
|------------------------------|----|
| Dow D.E.R. 332 (resin) ----- | 40 |
| Dimethyl formamide -----     | 60 |

Example 125

40

|                              |    |
|------------------------------|----|
| Dow D.E.R. 332 (resin) ----- | 80 |
| Dimethyl formamide -----     | 20 |

Example 126

45

|                                       |    |
|---------------------------------------|----|
| Dow D.E.R. 332 (resin) -----          | 50 |
| Ethylene glycol monobutyl ether ----- | 50 |

Example 127

50

|                                       |    |
|---------------------------------------|----|
| Dow D.E.R. 332 (resin) -----          | 80 |
| Ethylene glycol monobutyl ether ----- | 20 |

Example 128

55

|                                       |    |
|---------------------------------------|----|
| Dow D.E.R. 332 (resin) -----          | 30 |
| Ethylene glycol monoethyl ether ----- | 70 |

Example 129

60

|                                       |    |
|---------------------------------------|----|
| Dow D.E.R. 332 (resin) -----          | 90 |
| Ethylene glycol monoethyl ether ----- | 10 |

Example 130

65

|                                       |    |
|---------------------------------------|----|
| Dow D.E.R. 332 (resin) -----          | 80 |
| Ethylene glycol monohexyl ether ----- | 20 |

Example 131

70

|                                        |    |
|----------------------------------------|----|
| Dow D.E.R. 332 (resin) -----           | 30 |
| Ethylene glycol monomethyl ether ----- | 70 |

Example 132

75

|                                        |    |
|----------------------------------------|----|
| Dow D.E.R. 332 (resin) -----           | 90 |
| Ethylene glycol monomethyl ether ----- | 10 |

Example 133

80

|                              |    |
|------------------------------|----|
| Dow D.E.R. 332 (resin) ----- | 70 |
| Ethyl lactate -----          | 30 |

Example 134

85

|                              |    |
|------------------------------|----|
| Dow D.E.R. 332 (resin) ----- | 30 |
| Toluene -----                | 70 |

Example 135

90

|                              |    |
|------------------------------|----|
| Dow D.E.R. 332 (resin) ----- | 80 |
| Toluene -----                | 20 |

18

Example 136

Percent

|                              |    |
|------------------------------|----|
| Dow D.E.R. 332 (resin) ----- | 30 |
| Tricresyl phosphate -----    | 70 |

Example 137

Percent

|                              |    |
|------------------------------|----|
| Dow D.E.R. 332 (resin) ----- | 70 |
| Tricresyl phosphate -----    | 30 |

Example 138

Percent

|                              |    |
|------------------------------|----|
| Dow D.E.R. 332 (resin) ----- | 30 |
| Xylene -----                 | 70 |

Example 139

Percent

|                              |    |
|------------------------------|----|
| Dow D.E.R. 332 (resin) ----- | 80 |
| Xylene -----                 | 20 |

Example 140

Percent

|                                                                                                |     |
|------------------------------------------------------------------------------------------------|-----|
| Dow D.E.R. 332 (resin) -----                                                                   | 100 |
| 1 Distinctness of the chemical watermark fair-to-good. Not as good as when solvent is present. |     |

Example 141

Percent

|                           |    |
|---------------------------|----|
| Crestoset M (resin) ----- | 55 |
| Dimethylacetamide -----   | 45 |

Example 142

Percent

|                                         |    |
|-----------------------------------------|----|
| Dow D.E.R. 667 (resin) -----            | 60 |
| Diethyleneglycol monomethyl ether ----- | 40 |

Example 143

Percent

|                           |    |
|---------------------------|----|
| Crestoset M (resin) ----- | 55 |
| Diacetin -----            | 45 |

Example 144

Percent

|                                         |    |
|-----------------------------------------|----|
| Crestoset M (resin) -----               | 55 |
| Diethyleneglycol monomethyl ether ----- | 45 |

Example 145

Percent

|                           |    |
|---------------------------|----|
| Crestoset M (resin) ----- | 55 |
| Monacetin -----           | 45 |

Example 146

Percent

|                           |    |
|---------------------------|----|
| Crestoset M (resin) ----- | 55 |
| Dipropylene glycol -----  | 45 |

45 In the above examples it is clear that not only a wide number of solvents can be used but also the proportional amount may range from zero to as high as 80% although the range of 10 to 70% is more preferable. Furthermore some of these compositions are currently used for chemical watermarking paper commercially using conventional printing machinery.

In all of these examples the blank paper product employed in applying the compositions to form chemical watermarks according to this invention was of the bond grade consisting of 25% cotton and 75% woodpulp. The apparent density of the blank paper stock was about 5.0 and its thickness about 4 mils. The resulting chemical watermarks possessed a high degree of transparency. Other types of paper sheet products such as commercial mimeograph, tracing and even newsprint were successfully chemical watermarked with many of these compositions according to the invention.

In the paper industry the terms "opaque" and "semi-opaque" can refer to varying levels of opacity, depending on the specific type of paper under discussion. For purposes herein, more definite meanings can be given these terms by the following explanation.

In the writing paper field, trade practice classifies an "opaque" sheet of bond paper as one of a standard weight (500 sheets cut 17 inches by 22 inches, weighing between 19.5 lbs. and 20.5 lbs.) having a TAPPI (Technical Association of the Pulp and Paper Industry) opacity in excess of 87%. This percent is the reciprocal of the transmission of monochromatic light passing through the paper and photometrically measured.

The less commonly used term "semi-opaque" is generally accepted by the trade as a standard weight sheet of bond paper having a TAPPI opacity somewhere between 87% and 65%.

Writing papers having a TAPPI opacity less than 65% are often referred to as "transparent." It will suffice to say that the lower the TAPPI opacity, the more often the trade refers to "transparency," and the closer the opacity is to 65%, the more often the trade uses the term "translucent." Translucent papers usually retain the more common characteristics of bond papers, such as formation and brightness, whereas transparent sheets most often have a more uniformly translucent fibre mass with considerably less brightness. This holds true whether the paper under discussion is made entirely of chemical wood pulp, a blend of chemical wood pulp and cotton or linen fibres.

Technically the term "translucent" usually implies that a ray of light passing through a material is diffused while the term "transparent" implies that a ray of light passing through is not diffused. Thus a translucent object may vary from opaque to transparent according to the magnitude of diffusion of light passing therethrough. However, for purpose of this discussion the term transparent is used to denote that the magnitude of diffusion of light passing through the paper is not greater than that found in commercial tracing paper. Thus if a sheet of paper possesses a TAPPI opacity of less than 65% it is termed herein as "transparent" and conversely if 65% or greater it is termed herein as "translucent."

It has thus been shown that ordinary grades of stationery can be provided with a chemical watermark by a curable chemical impregnation according to this invention by means of a simple hand method or commercial printing machines. In commercial printing machines the compositions of this invention are employed instead of printing inks and may be applied in a similar manner as that described in my abovementioned co-pending application. From this it can be readily appreciated that small quantities of paper may be provided with a chemical watermark of selected configuration or design at costs which meet requirements of smaller volume customers and thereby making available, economically, a long sought paper product.

Based on the weight of paper the amount of curable impregnating composition of this invention, in terms of percent by weight, may vary due to the density of the paper and its impregnating characteristics. Therefore a sufficient amount effective to reduce the TAPPI opacity to below 65% is employed when working with translucent paper. In relation to the bond paper used in the examples, an impregnation in the amount of about 15% or less by weight of the resin based on the weight of the paper within the area impregnated gave satisfactory results.

Having thus described several embodiments of the invention it can now be seen that the objects of the invention have been fully achieved and it must be understood that changes and modifications may be made which do not depart from the spirit of the invention nor from the scope thereof as defined in the appended claims.

What is claimed is:

1. A method of imparting a chemical watermark of selected design to a finished sheet of paper which comprises the steps of printing the design on a portion of the surface of said paper sheet with a liquid composition consisting essentially of a synthetic, thermosetting, curable resin and an organic solvent, and removing said solvent to obtain a substantially colorless chemical watermark of

said deposited resin having an index of refraction of about 1.4 to about 1.7, and said chemical watermark being substantially free from gloss, having ink receptivity and resisting discoloration with aging substantially in the same way as the paper.

5 2. A method of imparting a chemical watermark of selected design to a finished sheet of paper which comprises the steps of printing the design on a portion of the surface of said paper sheet with a liquid composition consisting 10 essentially of synthetic, thermosetting curable resin and up to about 60% by weight of a curing agent for said resin, and hardening the composition by curing the resin to obtain a substantially colorless, chemical watermark having an index of refraction of about 1.4 to about 1.7, and said 15 chemical watermark being substantially free from gloss, having ink receptivity, and resisting discoloration with aging in substantially the same way as the paper.

20 3. A paper article with a chemical watermark which includes, in combination, a paper sheet, a chemical watermark composition applied on said sheet in the configuration of a selected design, the chemical watermarking composition consisting essentially of a hardened, synthetic, thermosetting resin having an index of refraction of about 1.4 to about 1.7, and said chemical watermark being substantially free from gloss, having ink receptivity and resisting discoloration with aging substantially in the same way as the paper.

25 4. An article as in claim 3 further characterized in that the resin is an epoxy resin.

5. An article as in claim 3 further characterized in that the resin is a melamine formaldehyde resin.

6. An article as in claim 3 further characterized in that the resin is a urea-formaldehyde resin.

30 7. An article as in claim 3 further characterized in that the resin is a polyester resin.

8. A paper article with a chemical watermark which includes, in combination, a paper sheet, a chemical watermark composition printed on said sheet in the configuration of a selected design, the chemical watermarking composition consisting essentially of a hardened, synthetic, thermosetting resin having an index of refraction of about 1.4 to about 1.7, and said chemical watermark being substantially free from gloss, having ink receptivity and resisting discoloration with aging substantially in the same way as the paper.

35 45

#### References Cited in the file of this patent

#### UNITED STATES PATENTS

|    |           |                       |                |
|----|-----------|-----------------------|----------------|
| 50 | 1,479,337 | Temple -----          | Jan. 1, 1924   |
|    | 1,998,237 | Himmell -----         | Apr. 16, 1935  |
|    | 2,285,095 | Rothrock et al. ----- | June 2, 1942   |
|    | 2,620,316 | Ritson -----          | Dec. 2, 1952   |
|    | 2,642,390 | Garofano -----        | June 16, 1953  |
|    | 2,683,089 | Reynolds -----        | July 6, 1954   |
| 55 | 2,721,505 | Mossberg -----        | Oct. 25, 1955  |
|    | 2,872,428 | Schroeder -----       | Feb. 3, 1959   |
|    | 2,888,452 | Schmid et al. -----   | May 26, 1959   |
|    | 2,900,364 | Wasserman -----       | Aug. 18, 1959  |
| 60 | 2,904,447 | Hochuli et al. -----  | Sept. 15, 1959 |

#### FOREIGN PATENTS

|         |                     |               |
|---------|---------------------|---------------|
| 696,673 | Great Britain ----- | Dec. 22, 1950 |
|---------|---------------------|---------------|

#### OTHER REFERENCES

65 The Condensed Chemical Dictionary, Reinhold Publishing Corp., Sixth Edition, New York, p. 1064, QD5C5, 1961, C. 6.